

## PHOTOGRAPHIC ANTIHALATION AND PROTECTIVE LAYER COMPRISING A NITRATED STYRENE-MALEIC ACID COPOLYMER

René Maurice Hart, Wilrijk-Antwerp, and Laurent Pierre Roosens and Jacques René Troquet, Antwerp, Belgium, assignors to Gevaert Photo-Producten N.V., Antwerp, Belgium, a Belgian company

No Drawing. Filed Nov. 26, 1957, Ser. No. 698,902

Claims priority, application Belgium Nov. 26, 1956

7 Claims. (Cl. 96—84)

The present invention relates to a photographic element provided with an alkali soluble hydrophobic outer layer containing as the main constituent a layer-forming polymer, and more particularly to a photographic element provided with an antihalation backing or with a protective layer applied to the light-sensitive silver halide layer or to the layer bearing already a silver image or a color image.

It is known to provide photographic elements such as black-and-white films and multilayer color films with an antihalation backing in order to inhibit light reflection from the back side to the emulsion side. This layer generally consists of a binding agent such as gelatin or a synthetic polymer, and a substance absorbing the light rays of this region of the spectrum to which the silver halide emulsion (or, in the case of a multilayer film, the emulsion layer nearest to the support) is sensitive.

It is further known to apply a protective layer (e.g. an anti-abrasive layer or a layer which absorbs the ultra-violet radiations) consisting of a layer-forming polymer to the light-sensitive layer (no the sensitive layers) or to a layer bearing already a silver image or a color image.

The polymeric products which are to be used as binding agents in outer layers such as the above-mentioned antihalation or protective layers must meet several severe requirements. Besides the particular function of these layers, they must in any case, on account of their position, possess special mechanical properties and show a resistance to outer influences such as friction, pressure, water, moist air etc. so that the films, plates or photographic papers provided with such layers can be treated in the processing baths and/or in the apparatus, e.g. cameras or projection apparatus, without being damaged.

If these layers must be applied to a flexible support, the layer-forming polymers must moreover be chosen in such a way that the formed layers possess a sufficient flexibility. Another requirement which particularly concerns the antihalation layers consists therein that neither this layer nor a constituent thereof may be transferred onto the silver halide emulsion layer if the emulsion layer and the backing layer come into contact e.g. when a photographic film is wound.

If it is desired that the layers are to be removed during the treatment in the usual photographic baths (e.g. in the case of antihalation layers containing a light-absorbing substance which is not or not completely decolorized in the processing baths), the polymeric binding agent must moreover be sufficiently soluble in the developers, which frequently are only slightly alkaline. On the other hand, the sensitivity to the alkali must not be too high since the contact of these layers e.g. with wet hands would damage the photographic element. A further requirement is that the layers obtained from the polymeric binding agent must be become sticky in moist atmosphere.

The derivatives of the styrene-maleic acid copolymers

which hitherto have been proposed as binding agent for antihalation layers do not possess the required properties. In moist atmosphere these layers become smooth and sticky, which involves a transfer of the colored particles of the antihalation layer onto the emulsion layer on winding and on storing the photographic element.

It is therefore an object of the present invention to provide new and improved antihalation coatings and protective layers. Another object is to provide such layers the flexibility of which is perfectly adapted to that of the usual flexible photographic supports to which they are to be applied. Another object of the invention is to provide antihalation coatings and protective layers which possess outstanding mechanical properties, such as an exceptional resistance to scratching and improved gliding properties. A further object is to provide such antihalation coatings which can be removed readily by weakly alkaline solutions such as the usual photographic developers. A still further object of our invention is to provide antihalation coatings and protective layers with hydrophobic character which possess exceptional resistance to moisture.

The above objects are accomplished in accordance with the present invention when the antihalation coating or the protective layer contains as the main constituent a nitrated styrene-maleic acid copolymer.

In order to obtain antihalation layers according to the present invention, an organic dyestuff or a mixture of such dyestuffs dissolved in an appropriated solvent can be incorporated in a solution of a nitrated styrene-maleic acid copolymer. Suitable antihalation dyestuffs can be found e.g. among the styryl dyestuffs, the tri- and di-aryl methane dyestuffs and the azomethine dyestuffs. The antihalation layer can be applied to a usual support such as e.g. to a flexible light-transmitting film support or to a glass plate, which is to be provided on the other side with a light-sensitive silver halide emulsion layer.

According to another embodiment of the present invention, antihalation layers can be prepared by starting from pigment dispersions e.g. carbon black in the polymeric binding agent. In this respect the nitrated styrene-maleic acid copolymers possess the great advantage to give stable dispersions by simply mixing, whilst stirring, the pigment with a solution of the polymer in an organic solvent such as a lower alcohol, without any addition of a dispersing agent. It is to be noted that the preparation of such dispersions with the polymers as used hitherto for the same purposes always necessitates an intense mechanical treatment, e.g. in a colloid mill. The black dispersion can be applied as antihalation coating to a suitable support as described hereinbefore.

When the nitrated styrene-maleic acid copolymers are to be applied as a protective layer on a light-sensitive emulsion layer or on a photographic image-bearing layer, especially a color image-bearing layer, ultra-violet radiation absorbing substances, such as diaminostilbene derivatives, derivatives of coumarone, pyrazoline or imidazoline, may be incorporated in the solution of the polymer. The support for the emulsion layer or for the image-bearing layer can be e.g. a flexible film or a baryta-coated paper.

The nitrated styrene-maleic acid copolymers are obtained by action of nitric acid upon styrene-maleic acid copolymers. Although in general fuming nitric acid hitherto was used therefor, a great part (up to 70%) of the fuming nitric acid can be replaced by ordinary nitric acid. In the circumstances the reaction runs very smoothly at room temperature. Also a mixture of nitric acid and sulphuric acid can be used. In the event, the reaction is better carried out whilst heating e.g. between 50 and 70° C. Also the proportion nitric acid/sulphuric acid is of importance and the best results are

attained with proportions ranging from 7/3 to 9/1. In this way about one nitrogroup per styrene unit is incorporated, which theoretically corresponds with a nitrogen content of 5.3%.

The degree of polymerization of the starting products is only slightly influenced by the nitration. This degree of polymerization is not of particular importance in the preparation of ordinary antihalation layers with soluble dyestuffs, but must be taken into account in the preparation of antihalation backings containing carbon black. In this case, polymers with a relatively low molecular weight are preferably used so that strongly concentrated solutions (25 to 35%) can be prepared which do not show an excessive viscosity.

Hereinafter follow some examples of preparing the nitrated styrene-maleic acid copolymers.

#### PREPARATION 1

##### (a) Styrene-maleic acid copolymer

41.6 parts by weight of styrene (previously washed with a solution of sodium hydroxide and water respectively, dried upon calcium chloride and distilled in nitrogen atmosphere under reduced pressure) are copolymerized with 43.1 parts by weight of maleic acid anhydride in 730 parts by volume of toluene, previously dried upon calcium chloride. The mixture is heated at 110° C. for 9 hours in the presence of 0.42 part by weight of azobisisobutyronitrile as initiator. The polymerization mixture is filtered and the deposited styrene-maleic acid copolymer is washed with hexane and dried in a desiccator at 50° C.

##### (b) Nitrated styrene-maleic acid copolymer

80 parts by weight of a styrene-maleic acid copolymer are dissolved whilst stirring in 400 parts by volume of fuming nitric acid, whilst the temperature is kept below 10° C. by ice-cooling.

The clear solution is precipitated in distilled water. The precipitate is pulverized and washed with distilled water to neutral reaction as can be controlled with indicator paper. The product is dried under vacuum at 40° C. It contains 5.6% of nitrogen.

#### PREPARATION 2

350 cm.<sup>3</sup> of strong nitric acid ( $d=1.42$ ) and 150 cm.<sup>3</sup> of fuming nitric acid ( $d=1.52$ ) are brought into a reaction flask, and 100 g. of styrene-maleic acid copolymer are gradually added whilst stirring at a temperature kept between 25 and 30° C. After standing overnight the solution is added to water and the formed precipitate is washed with water.

The product is dried under vacuum to constant weight. It contains 5.4% of nitrogen.

#### PREPARATION 3

A nitrated styrene-maleic acid copolymer is prepared by causing 1 kg. of the styrene-maleic acid copolymer to react with 6.3 liter of strong nitric acid ( $d=1.42$ ) and 0.95 liter of sulphuric acid (96%) for 8 hours at 60° C.

The formed reaction product is separated in the same way as in the previous examples. It contains 5.5% of nitrogen.

The following examples illustrate the invention without limiting, however, the scope thereof.

#### EXAMPLE 1

A solution of 60 g. of a nitrated styrene-maleic acid copolymer in a mixture of 300 cm.<sup>3</sup> of ethanol and 300 cm.<sup>3</sup> of methanol is prepared. This solution (hereinafter called A) is added to a solution of 22 g. of a green dyestuff (known under the denomination Bro 721 and described in BIOS comp. 146/2/382/30), in a mixture of 200 cm.<sup>3</sup> of ethanol and 200 cm.<sup>3</sup> of methanol (solution B). This solution is coated on the rear of a cellulose acetate-butylate film support, the front side of which is to be provided with a panchromatic sensitized silver iodide

bromide emulsion. After evaporation of the solvents an intense-green colored layer is obtained which possesses very good mechanical properties and which loses its absorption power in the ordinary photographic processing baths.

#### EXAMPLE 2

22 g. of a dyestuff of the following formula



are dissolved in a mixture of 200 cm.<sup>3</sup> of ethanol and 200 cm.<sup>3</sup> of methanol. This colored solution is added to solution A described in Example 1. After application to the rear of a cellulose triacetate film support which is to be provided with an orthochromatic sensitized silver chloro-bromide emulsion, a deep-red colored layer is obtained which loses its absorption power in the ordinary photographic treating baths and dissolves completely therein.

#### EXAMPLE 3

10 g. of a dyestuff of the following formula:



are dissolved in a mixture of 200 cm.<sup>3</sup> of ethanol and 200 cm.<sup>3</sup> of methanol. This solution is added to the solution A described in Example 1. After application to a suitable support in the manner described in Example 2, an orange-colored layer is obtained which decolorizes in the processing baths.

#### EXAMPLE 4

22 g. of a dyestuff described in PB report 74174, frame 45 820 (U.S. Government, Office of Technical Services, Washington), are dissolved together with 60 g. of nitrated styrene-maleic acid copolymer in a mixture of 500 cm.<sup>3</sup> of ethanol and 500 cm.<sup>3</sup> of methanol. After application to a flexible support which is to be provided with three differentially sensitized silver halide emulsion layers containing color couplers, a violet layer is obtained. This layer decolorizes and dissolves in the photographic processing baths.

#### EXAMPLE 5

55 7 g. of carbon black are added to a solution of 60 g. of a nitrated styrene-maleic acid copolymer in 250 cm.<sup>3</sup> of ethanol, whilst thoroughly stirring. After dispersing the carbon black, the volume is brought to 1 liter by adding a mixture of 1 part of ethanol and 2 parts of methanol. This solution can be cast onto a flexible support. A brown-black layer is obtained which is easily removable in photographic processing baths. The light-reflection being almost completely inhibited by this layer, a photographic element e.g. a positive motion picture color film, provided therewith, is free from halation.

#### EXAMPLE 6

70 A solution of 9 g. of a nitrated styrene-maleic acid copolymer in a mixture of 700 cm.<sup>3</sup> of ethanol and 300 cm.<sup>3</sup> of methanol is coated as an anti-abrasive layer onto a silver chloro-bromide emulsion layer on a baryta-coated paper support. The photographic properties of the light-sensitive layer do not markedly change even during long periods of stockage, and moreover the friction fog is

considerably diminished in respect of those of a photographic emulsion without protective layer.

## EXAMPLE 7

75 g. of a nitrated styrene-maleic acid copolymer and 5 g. of Teregitol NP 35 (trademark for alkylphenylpolyethylene glycol ether) are dissolved in a mixture of 600 cm.<sup>3</sup> of ethanol, 160 cm.<sup>3</sup> of ether, 100 cm.<sup>3</sup> of isopropylalcohol and 50 cm.<sup>3</sup> of methylene-glycol. This solution is mechanically applied to the image-bearing layer of an exposed and developed motion picture film of the positive type. This layer protects the film against scratching, moisture and mishandling during the treatment.

## EXAMPLE 8

12 g. of "Uvinul 400" (a substituted benzophenone) are added the solution of the copolymer described in Example 6. This solution is applied as protective layer on the emulsion layer of a photographic negative film. This layer protects the emulsion against ultra-violet rays.

We claim:

1. A photographic element comprising a support, at least one light-sensitive silver halide emulsion layer, and an alkali-soluble hydrophobic outer layer, said outer layer being mainly constituted by a nitrated copolymer consisting of 50 mol percent styrene monomeric units alternating with 50 mol percent maleic acid monomeric units, the copolymer containing 0.8 to 1.2 nitro groups per styrene monomeric unit.

2. A photographic element comprising a flexible light-transmitting support, at least one light-sensitive silver halide emulsion layer on one side of said support, and an alkali-soluble hydrophobic anti-halation layer on the other side of said support, said anti-halation layer comprising a copolymer and a light-absorbing substance, said copolymer consisting of 50 mol percent styrene monomeric units alternating with 50 mol percent maleic acid monomeric units, the copolymer containing 0.8 to 1.2 nitro groups per styrene monomeric unit.

3. The photographic element according to claim 2, wherein the light-absorbing substance is an organic dye-stuff.

4. The photographic element according to claim 2, wherein the light-absorbing substance is carbon black.

5. A photographic element comprising a support, at least one light-sensitive silver halide emulsion layer on one side of said support, and an alkali-soluble hydrophobic protective layer coated on said emulsion layer, 10 said protective layer being mainly constituted by a copolymer consisting of 50 mol percent styrene monomeric units alternating with 50 mol percent maleic acid monomeric units, the copolymer containing 0.8 to 1.2 nitro groups per styrene monomeric unit.

15 6. The photographic element according to claim 5, wherein the protective layer includes an ultra-violet radiation absorbing substance.

7. A photographic element comprising a support, at least one image-bearing layer, said image having been 20 obtained by exposing to light a light-sensitive silver halide emulsion layer on one side of said support, said element further comprising a protective layer coated on said image-bearing layer, said protective layer being mainly constituted by a copolymer consisting of 50 mol percent 25 styrene monomeric units alternating with 50 mol percent maleic acid monomeric units, the copolymer containing 0.8 to 1.2 nitro groups per styrene monomeric unit.

## References Cited in the file of this patent

## UNITED STATES PATENTS

|              |               |       |                |
|--------------|---------------|-------|----------------|
| 2,077,789    | Hagedorn      | ----- | Apr. 20, 1937  |
| 2,173,480    | Jung          | ----- | Sept. 19, 1939 |
| 2,274,551    | Kenyon et al. | ----- | Feb. 24, 1942  |
| 35 2,685,512 | Sawday        | ----- | Aug. 3, 1954   |
| 2,748,029    | Spear et al.  | ----- | May 29, 1956   |

## FOREIGN PATENTS

|         |           |       |               |
|---------|-----------|-------|---------------|
| 115,781 | Australia | ----- | Aug. 25, 1942 |
|---------|-----------|-------|---------------|

UNITED STATES PATENT OFFICE  
CERTIFICATE OF CORRECTION

Patent No. 2,984,568

May 16, 1961

René Maurice Hart et al.

It is hereby certified that error appears in the above numbered patent requiring correction and that the said Letters Patent should read as corrected below.

Column 1, line 35, for "no" read -- or --; same column, line 70, for "be" read -- not --.

Signed and sealed this 21st day of November 1961.

(SEAL)

Attest:

ERNEST W. SWIDER

Attesting Officer

DAVID L. LADD

Commissioner of Patents

USCOMM-DC